

# UNITED STATES PATENT OFFICE.

WILLIAM AUGUSTUS HALL, OF NEW YORK, N. Y.

## PROCESS FOR THE EXTRACTION OF SULFUR FROM METALLIC SULFIDS.

1,083,248.

Specification of Letters Patent.

Patented Dec. 30, 1913.

No Drawing.

Application filed October 10, 1912. Serial No. 725,024.

To all whom it may concern:

Be it known that I, WILLIAM AUGUSTUS HALL, a citizen of the United States Republic, and resident of New York, N. Y., 5 United States of America, have invented a certain new and useful Improvement in Processes for the Extraction of Sulfur from Metallic Sulfids, of which the following is a specification.

10 This invention relates to an improvement in the process described in the specification of my co-pending application for patent Serial Number 725,026, filed concurrently herewith. In the specification accompanying that application I described a process of producing sulfureted hydrogen from metallic sulfids *e. g.* iron pyrites by submitting the pyrites to the combined action of a reducing flame (which decomposes it without producing any appreciable oxidation) and steam intended to furnish nascent hydrogen and nascent oxygen for the purposes described in said application, the operations being carried out under such conditions that 25 fresh surfaces of the pyrites are continuously exposed to the action of the reducing flame and of the steam.

The object of my present invention is to extract the sulfur from pyrites or other 30 sulfid ores, principally in the form of elemental sulfur, and not principally in the form of  $H_2S$ , as in the process of my other application above referred to.

In the practice of the prior process referred to, I employed in conjunction with the direct reducing flame a considerable amount of steam in order that the nascent hydrogen thereof would combine with the sulfur vapor to form  $H_2S$  and that the 40 nascent oxygen of the steam would supply a stable equivalent to the iron of the pyrites.

In accordance with the present process I supply to the furnace in conjunction with the direct reducing flame a very small 45 amount of steam, so small in amount that without the flame substantially no decomposition of the pyrites would take place yet sufficient in amount to prevent substantial loss of sulfur by formation of  $SO_2$  and 50 of  $CO_2$ .

By using a small amount of steam in accordance with this invention I am also enabled to admit more air with the "gaz pauvre" or producer gas than would be

practicable were no steam used, thus permitting a more perfect combustion and higher temperature with less volume of gas and without loss from the  $SO_2$  formation. The temperature in the present process is, by means of limiting the amount of steam, 55 maintained at or above the temperature at which sulfur distils from the ore, namely at or about  $700^{\circ} C.$ , and preferably between 60  $700$  and  $900^{\circ} C.$  At these temperatures, and by the action of a reducing flame, the principal part of the sulfur of the pyrites, or other sulfid ore, is driven off in the form of elemental sulfur, directly by distillation, and the remainder of the sulfur is driven off from the pyrites by reaction with the 65 steam to produce  $H_2S$ . If this proper amount of air were admitted without any steam, then the discharge would contain a considerable amount of  $SO_2$  which might be lost; but by admitting the steam, the  $SO_2$ , 70 formed is taken care of by the  $H_2S$  also formed, in accordance with the well known equation  $2H_2S + SO_2 = 3S + 2H_2O$  and the sulfur precipitated thereby is carried over 75 with the sulfur vapor and deposited therewith. In this way the steam takes care of any excess air that may pass into the furnace and intended for the perfect combustion of the "gaz pauvre."

In accordance with the practice of my invention I take a furnace preferably of any well known mechanical type such as described for instance in the specification of my co-pending application Serial Number 725,023, filed concurrently herewith (wherein much agitation of the pyrites may be effected) heated internally by direct flame produced from a mixture of "gaz pauvre" or producer gas and air, the amount of air admitted being so regulated that the flame 85 produced while not necessarily a highly reducing flame, is of sufficient reducing character to combine with any free oxygen. Steam, or water which would be transformed into steam, is passed in through 90 inlets suitably disposed, preferably in larger quantity toward the lower end of the furnace, the furnace being provided with a gas outlet from which extends a long discharge pipe. Into this discharge pipe steam 95 may also be passed with the object herein-after referred to. When the furnace has been raised to the proper degree of temper-

ature preferably somewhat above 700° C. the distilling temperature of the sulfur of the pyrites, the pyrites is led thereinto in a continuous stream with the least admission 5 of air possible.

I find it desirable at all times to maintain a very slight internal pressure in the furnace which is easily accomplished by means of the expanded gases. This prevents ingress of 10 any undesirable excess air.

It is essential that the pyrites should be agitated to the greatest possible extent while in the furnace. If this were not done much less sulfur would be discharged. The products 15 of combustion pass up through the long pipe in which the temperature is reduced several hundred degrees and the products of combustion pass out surcharged with yellow sulfur vapor without any appreciable 20 admixture of  $\text{SO}_2$ . This fact has been determined by analysis of the gases. The discharge pipe leads the sulfur vapor and products of combustion to a gas-washing apparatus such as the well known Thiesen apparatus 25 where the atmosphere is quickly clarified by the precipitation of the finely divided sulfur in the water of the washer and from this it is extracted by any desired means.

30 The reactions that take place in the interior of the furnace are:—(1) A decomposition of the pyrites  $\text{FeS}_2$  and distillation of sulfur in the form of sulfur vapor a small portion of which may combine with any excess oxygen present. Very much over one-half of the total sulfur in the pyrites can be distilled off without first being converted into  $\text{H}_2\text{S}$  and  $\text{SO}_2$ . (2) A decomposition of the steam by the lower sulfids of iron, while 35 at a high temperature forming  $\text{H}_2\text{S}$ ,  $\text{Fe}_2\text{O}_3$  and some  $\text{Fe}_3\text{O}_4$ . (3) The combination of this  $\text{H}_2\text{S}$  with any  $\text{SO}_2$  present, forming elemental sulfur by the well known reaction  $2\text{H}_2\text{S} + \text{SO}_2 = 2\text{H}_2\text{O} + 3\text{S}$  which sulfur is carried 40 over to the condenser along with the distilled sulfur and products of combustion and (4) the formation of COS from some of the excess of CO contained in the "gaz pauvre" or producer gas. This would ordinarily cause a considerable loss in sulfur. I meet this difficulty by admitting more steam which may be passed into the discharge pipe as already described, where at 45 lower temperatures it combines with the COS forming  $\text{H}_2\text{S}$  and  $\text{CO}_2$ ; this  $\text{H}_2\text{S}$  also combines with excess of  $\text{SO}_2$  in the same manner as does the  $\text{H}_2\text{S}$  generated in the furnace as hereinbefore described.

Without steam there is a tendency for the 50 iron sulfids to fuse slightly and for the particles of pyrites to adhere together but this is largely overcome by the admission of the small amount of steam and by the continuous agitation. The decomposition of the 55  $\text{H}_2\text{O}$  of the steam by the hot iron forms

$\text{Fe}_2\text{O}_3$  and thus tends to break down and disintegrate the coarser pieces of the pyrites.

While I have described my process in detail as applied to the treatment of pyrites, it is to be noted that this process is as stated above, useful in connection with sulfid ores generally, and is not restricted to the treatment of pyrites. Among the other materials which I have treated according to this process, are pyrrhotite and artificial ferrous sulfid ( $\text{FeS}$ ). Even when using these materials, which contain much less sulfur than does pyrites, I can remove the major portion of the sulfur therefrom by direct distillation.

It will be seen that in my process, a large part of the sulfur is driven off from the pyrites in the form of free or elemental sulfur, and not as compounds thereof,  $\text{SO}_2$  and  $\text{H}_2\text{S}$ , as in some of the processes heretofore proposed. The cause of this is the fact that a reducing flame, in contact with the ore, is employed, together with the fact that a small amount of steam is admitted.

The removal of both fixed and feeble 90 atoms of sulfur, from sulfid ores broadly, and specifically from those varieties of sulfid ore which do not contain any material amount of pyrites or other ore containing both fixed and feeble atoms of sulfur, is not 95 claimed herein, but forms the subject matter of my copending application Serial No. 770,946, filed May 31, 1913.

Having described my invention what I claim and desire to secure by Letters Patent 100 of the United States is:—

1. In the production of sulfur from ores containing considerable amounts of pyrites, subjecting said ore to the action of a reducing flame and of a limited amount of steam 105 which amount is in itself insufficient to produce considerable amounts of  $\text{H}_2\text{S}$ , but sufficient to prevent substantial loss of sulfur due to formation of material quantities of  $\text{SO}_2$  and COS.

2. A process of extracting sulfur from metallic sulfids, containing considerable amounts of pyrites, which comprises agitating the sulfid and simultaneously subjecting the same to the combined action of a direct 110 reducing flame and of a small amount of  $\text{H}_2\text{O}$ .

3. A process of extracting sulfur from those sulfid ores which contain considerable quantities of sulfid containing both fixed and feeble atoms of sulfur, which comprises subjecting such sulfids to the simultaneous action of a reducing flame and of a relatively small volume of steam while causing fresh surfaces of the sulfids to be exposed 120 throughout the operation.

4. A process of extracting sulfur from metallic sulfids, which comprises subjecting the sulfids to the action of steam and of a reducing flame produced by combustion of 125

producer gas, reacting with steam on any carbon oxy-sulfid that may be formed to produce sulfureted hydrogen and carbon dioxid and reacting on the sulfureted hydrogen with sulfur dioxid to precipitate sulfur.

5. A process of extracting sulfur from metallic sulfids which comprises agitating the sulfids and simultaneously subjecting the 10 same to the combined action of a direct reducing flame and of a small amount of steam, while maintaining the gases evolved at a pressure exceeding normal atmospheric pressure.
15. 6. In the production of free sulfur from sulfid ores, containing considerable quantities of pyrites, the step of subjecting a layer of said ore, to the action of a reducing flame, and of steam, while agitating said 20 ore.
7. In the production of free sulfur from pyrites ore, the step of subjecting a layer

of said ore, to the action of a reducing flame, together with a small amount of steam.

8. In the production of free sulfur from 25 ores containing pyrites, the step of subjecting a layer of said ore, to the action of a reducing flame, at a temperature at which free sulfur distils from said ore.

9. In the production of free sulfur from 30 sulfid ores containing pyrites, the step of subjecting a layer of said ore, to the action of a reducing flame, together with sufficient steam to prevent the formation of material amounts of  $\text{SO}_2$ , and to decompose any  $\text{CO}_2$  35 formed.

In testimony whereof I have signed my name to this specification in the presence of two subscribing witnesses.

WILLIAM AUGUSTUS HALL.

Witnesses:

HAROLD G. C. FAIRWEATHER,  
ALFRED T. BURBERRY.